

Sept. 1, 1925.

1,552,040

F. F. FOWLE ET AL

PROTECTED METAL AND PROCESS OF MAKING IT

Filed Dec. 18, 1923



Patented Sept. 1, 1925.

1,552,040

# UNITED STATES PATENT OFFICE.

FRANK F. FOWLE, OF KENILWORTH, ILLINOIS, AND FREDERICK M. CRAPO, OF MUNCIE, INDIANA.

## PROTECTED METAL AND PROCESS OF MAKING IT.

Application filed December 18, 1923. Serial No. 681,435.

To all whom it may concern:

Be it known that we, FRANK F. FOWLE and FREDERICK M. CRAPO, citizens of the United States, residing at Kenilworth, in the county of Cook, Illinois, and at Muncie, in the county of Delaware and State of Indiana, respectively, have invented a new and useful Protected Metal and Process of Making It, of which the following is a specification.

The primary object of our invention is to improve the zinc-coating of iron and low-carbon steel articles, especially of iron and steel wire. More specifically, such primary object is to produce a zinc-coated article, especially iron or low-carbon steel wire, the coating of which will adhere firmly and will not peel or flake off even when subjected to sharp bends or twists, as for example upon wrapping such a wire around its own diameter; and especially to accomplish all this effectively with iron or low-carbon steel.

It is our further object to get this improved zinc-coating without substantially impairing the mechanical and electrical properties of such coated articles, especially wire, such as tensile strength, elongation and electrical resistivity.

Still another object of our invention is to produce a more satisfactory and enduring zinc-coating with a smaller quantity of zinc.

In accomplishing these results, from the standpoint of zinc-coating, we first coat the iron-base article, such as iron or low-carbon steel wire, advantageously before it has been drawn to finished size, with a thin layer or film of relatively high-carbon steel; and subsequently apply the zinc coating. The first coating or jacket of relatively high-carbon steel is a binder, and serves to improve the bond between the iron or low-carbon steel core and the zinc coating.

We recognize as prior art the co-pending application of one of us, Frederick M. Crapo, Ser. No. 679,650, filed Dec. 10, 1923, now Patent No. 1,501,887, granted July 15, 1924.

We also recognize as independent inventions of said Frederick M. Crapo certain things specifically claimed by him in certain co-pending applications filed by him, as follows:

Serial No. 695,423, filed February 27, 1924;

Serial No. 712,000, filed May 9, 1924; and

Serial No. 744,976, filed October 21, 1924.

The accompanying drawings illustrate our

invention: Fig. 1 is a greatly magnified fragmental cross-section of a wire coated in accordance with our invention; Fig. 2 is a more highly magnified fragmental cross-section of such wire, to indicate the alloy films formed in the coating process; Fig. 3 is a vertical section through an ingot mold in which the steel coating is obtained by pouring molten steel around an iron core; Fig. 4 is a vertical section through an ingot mold in which the coating of steel on the iron core is obtained by pouring the molten iron within a steel tube which lines the mold and eventually forms the jacket or coating of the ingot; Figs. 5 and 6 are vertical sections through a bath of molten steel for steel-coating dipped-in ingots and wire respectively; and Fig. 7 is a diagrammatic view illustrating the general sequence of operations on a steel-coated billet to produce a zinc-coated wire therefrom.

The essence of our invention is a plurality of coatings on an iron-base (or ferrous metal) article 10, especially iron or low-carbon steel, chief in which are a coating or jacket of relatively high-carbon steel 11 and a coating of zinc 12, applied and existing in the order named; as is shown in Fig. 1.

We recognize that in the process of applying the high-carbon steel coating, and in the hot-process of applying the zinc coating, intermediate coatings or films of alloy of the coated metal and the coating material inherently will be formed and will exist in the final product; as is illustrated in Fig. 2. For example, there will be an intermediate alloy film 13 of iron and steel, or of low-carbon steel and high-carbon steel, between the primary iron-base body and the high-carbon steel coating; and there may be present a plurality of such intermediate alloy films, graduated in composition from the constituents of the iron-base body to the constituents of the steel coating. Likewise there will be an intermediate coating or alloy film 14, between the high-carbon steel coating and the zinc coating, comprising an alloy of steel and zinc, or of iron, steel and zinc, or of iron and zinc, or a plurality of such alloys; and there may be present a plurality of such intermediate alloy films, of various intermediate compositions.

We do not limit ourselves to the hot processes of applying zinc coatings, known to the art, but we may also use the electro-

galvanic process, or this process in combination with subsequent hot process. This is shown in Fig. 7, where the bath 15 is an electro-galvanic zinc-plating bath of any convenient type, and the bath 16 is a bath of molten zinc for the hot-process application of a zinc coating. However we prefer the hot process alone, because of the attendant advantage we secure in the contemporaneous annealing action on the steel coating and the iron-base body and their intermediate film of alloy. By the term hot process of zinc coating we mean any of the known processes for applying zinc coatings which are dependent upon the application of heat to the article to be coated and to the coating material, including the use of cleaning and/or fluxing materials 17 and 18 for preparative purposes; and the use of neutral and/or reducing gases or atmospheres for the purpose of enveloping the iron-base body, or said body in combination with its steel coating, while in hot condition, and thus retarding or preventing surface oxidation of the same.

We do not limit ourselves to any one process for applying the coating of steel to the iron-base body, but we may use any known process for this purpose or suitable modification of known processes for coating one metal with another in the hot state of one or both. For example, as shown in Fig. 3, we can use the process of casting molten steel 20 around an ingot or bar of iron 21 which has been suitably cleaned, fluxed, pre-heated and inserted in a suitable mold 22 of such dimensions with respect to the iron bar or ingot as to obtain a substantially uniform thin coating of steel enveloping the iron except at the supporting contacts 23 between the iron body and the mold. In this illustration the iron might be in the form of a cylindrical ingot, billet, or bar, placed in a cylindrical mold 22 so as to obtain a thin tubular coating or jacket 20 covering the outer curved surface of the iron body. We can also, as shown in Fig. 4, take a thin tube 24 of steel and suitably clean, flux and pre-heat it for use as the lining of a mold 25 to receive molten iron 26; and then pour molten iron into the interior of said mold until full, so that the iron will adhere to the inner surface of the lining 24 of the mold and when solidified become a single integral body. The steel-coated iron-base ingots, billets, or bars thus produced may be hot-rolled into rods and cold-drawn into wire by familiar processes in the art which require no detailed description, but are indicated diagrammatically in Fig. 7; or the steel-coated bars may be rolled into sheets, or hot-fabricated into pipes, by methods familiar to the arts; other shapes or products may be manufactured from these steel-coated iron-base bars, but in all the examples just cited it is intended that the ultimate prod-

uct may be a zinc-coated article, though if desired we may omit the zinc coating, and still obtain an article of value for many purposes and fairly resistant to corrosion.

We may also obtain a steel coating by the process of briefly hot-dipping an iron-base body in a bath of molten steel 30; and in the example of rods or wire 31 the process may be worked in continuous operation, as illustrated in Fig. 6. In the hot-dipping process, the iron-base body is suitably cleaned, fluxed and preheated, by well-known means, before dipping, so as to promote the alloying of the molten steel with the surface metal of the iron-base body and also for the purpose of promoting the adherence of an outer film of hot steel upon withdrawing the iron-base body from the molten bath. We prefer the method, illustrated in Fig. 5, of dipping the iron-base body 32, when in the form of an ingot, billet, bar, or rod, before subjecting the same to the process of cold working, such as cold rolling or cold drawing; and before hot-fabricating such billets or bars into pipe or other products requiring hot-working processes to manufacture them into final shape and size.

When the hot-dipping process is employed to steel-coat an iron-base body for manufacture into zinc-coated wire, the steel-coated billet 32, or steel-coated bar, for example, may be then hot-rolled into rods 33 and next cold-drawn into wire 34; and subsequently coated with zinc; as is illustrated in Fig. 7. If the hot-dip is applied to the rod, it may then be cold-drawn into wire; and a zinc coating subsequently applied.

By the use of the term carbon-steel we mean the commercial grades of steel commonly referred to as carbon-steel, in which the predominating ingredient is the element iron and the constituent of succeeding importance is a small quantity of the element carbon, in chemical combination with iron, or so-called combined carbon; small quantities of manganese and silicon are also usually present, and traces or slight impurities consisting of sulphur and phosphorus; in addition these steels sometimes contain very small ingredients of various non-ferrous metals added to the steel in the molten state for the purpose of deoxidizing it, or for improving its molten fluidity, or for promoting the formation of stable compounds upon passing from the hot fluid state to the cold solid state, or for rendering the steel product more resistant to corrosion, or for improving the general properties of the steel product, such as manganese, silicon, aluminum, chromium, vanadium, tungsten, nickel, copper, tin, titanium and molybdenum. As one example of carbon-steel which is rendered more resistant to corrosion we may mention the so-called copper-bearing steel which contains about one-

fourth of one per cent of copper. We recognize that the addition of substantial proportions of certain non-ferrous metals to steel, such as chromium, vanadium, or nickel for example, bring the product into the class commonly referred to as alloy-steels, but the use of such alloy steels in forming the steel coating before described is not an essential feature of our invention, as we prefer the use of steel coatings comprising the kind of material which is predominantly carbon-steel; for our purposes it would suffice even to use a crucible steel containing only the elements iron and carbon, aside from substantially irremovable impurities. We have not attempted to mention or describe all of the known or possible processes for coating an iron or relatively low-carbon steel body with relatively high-carbon steel and our invention is not limited to those processes which we have mentioned or described, but embraces every method of producing such coating and subsequently applying a coating of zinc. Furthermore it is not essential, in our invention, to obtain a coating of steel which is substantially thick, but the steel coating may be as thin as practicable, or, at the minimum, of the order of thickness of the intervening alloy films before described, which is the result that we prefer. It is also immaterial, in our invention, at what stage in the process as a whole the steel coating is applied, so long as it is applied before the coating of zinc is applied; and it is not necessarily a detriment to our product if the steel coating is applied two or more times, either in succession or not, or whether at the same stage or at different stages in the manufacture, but we prefer a single steel coating as sufficient to attain our result, and we also prefer, in the example of wire, to apply the steel coating before the operation of cold-drawing or else in the early stages of drawing, and especially by casting the iron or low-carbon steel in a relatively high-carbon steel tube.

We claim as our invention:—

1. A zinc-coated iron or steel article, comprising an iron or low-carbon steel body; and a plurality of separately applied coatings thereon, including a coating of zinc, and a coating of steel interposed between the zinc coating and the said body and of relatively high carbon content.

2. Zinc-coated iron or steel wire, comprising an iron or low-carbon steel core; and a plurality of separately applied coatings thereon, including a coating of zinc, and a coating of steel interposed between the zinc coating and the said core and of relatively high carbon content.

3. A zinc-coated iron or steel article, comprising an iron-base body having a relatively low carbon content, an iron-base

jacket or coating upon and adhering to said body and having a relatively high carbon content and an outer coating of zinc upon and adhering to said iron-base jacket or coating.

4. Zinc-coated iron or steel wire, comprising an iron-base core having a relatively low carbon content, an iron-base jacket or coating upon and adhering to said core and having a relatively high carbon content, and an outer coating of zinc upon and adhering to said iron-base jacket or coating.

5. The process of making zinc-coated wire, comprising making a relatively low-carbon iron-base core; and separately applying a plurality of adhering coatings thereon, including applying a relatively high-carbon iron-base coating as a binder and later applying a zinc-coating, so that the first coating serves to improve the bond between the core and the zinc coating.

6. The process of making zinc-coated iron-base wire, comprising rolling the rods from iron-base ingots of relatively low carbon content, and drawing the wire from such rods; incasing the wire stock at any desired time in an integrally adhering layer of iron-base material of relatively high carbon content as a binder; and applying a zinc coating to the incased wire, so that the binder layer serves to improve the bond of the zinc coating to the wire.

7. The process of making zinc-coated iron-base wire, comprising pouring ingots of iron or low-carbon steel in a tube of relatively high-carbon steel so that the tube forms an integrally adhering binder jacket or coating for the ingot; rolling the ingot into rods and drawing the rods into wire; and applying a zinc-coating to the wire so formed, so that the binder jacket or coating serves to improve the bond of the zinc coating to the wire.

8. The process of making zinc-coated iron or low-carbon steel wire, comprising rolling a base stock from the ingot to the rod; applying an integrally adhering iron-base binder jacket or coating of relatively high carbon content to the wire stock before it is reduced to the rod size, so that subsequent rolling will act on said jacket or coating as well as on the wire stock within it; subsequently drawing the wire from the rod; and applying a zinc coating to the wire, so that the binder jacket or coating serves to improve the bond of the zinc coating to the wire.

9. The process of making a zinc-coated article, comprising forming a core of iron or low-carbon steel; incasing said core in an integrally adhering iron-base binder jacket or coating of relatively high carbon content at any desired stage in its manufacture; and subsequently applying a zinc-

coating upon such iron-base coating or jacket, so that the binder jacket or coating serves to improve the bond of the zinc coating to the core.

10. The process of making a zinc-coated iron-base article, comprising casting an ingot of iron or low-carbon steel in a tube of relatively high-carbon steel so that the tube forms an integrally adhering binder coating or jacket for said ingot; operating on said ingot to increase its length and reduce its cross-section to desired shape and size; and applying a zinc-coating upon the article, so that the binder jacket or coating serves to improve the bond of the zinc coating to the iron-base article.
11. The process of making an iron-base

article, comprising casting an ingot of iron or relatively low-carbon steel; coating said ingot with a layer of relatively high-carbon steel as a binder; operating on said coated ingot to increase its length and reduce its cross-section to desired size and shape; and applying an outer coating of a non-ferrous metal to said article, so that the binder layer serves to improve the bond of the non-ferrous metal to the iron-base article.

In witness whereof, we have hereunto set our hands at Washington, D. C., this 18th day of December, A. D. one thousand nine hundred and twenty-three.

FRANK F. FOWLE.  
FREDERICK M. CRAPO.